

F. A. STIEF,

REFINING LEAD ALLOYS AND ALLOYS CONTAINING LEAD, TIN, COPPER, OR ANTIMONY.  
APPLICATION FILED MAY 6, 1915.

1,283,427.

Patented Oct. 29, 1918.

2 SHEETS—SHEET 1.



*Witnesses:*

Edgar T. Farmer.  
Austolcombe.

Inventor:  
W. Fred A. Steff,  
by Barr Stearn,  
his attorney.

F. A. STIEF.

REFINING LEAD ALLOYS AND ALLOYS CONTAINING LEAD, TIN, COPPER, OR ANTIMONY.  
APPLICATION FILED MAY 6, 1915.

1,283,427.

Patented Oct. 29, 1918.  
2 SHEETS—SHEET 2.

*Fig. 3.*



*Fig. 4.*



Witnesses:

Edgar T. Farmer,

Ames Holcombe

Inventor:

F. A. Stief,

by Carr & Carr,  
his Atty's.

# UNITED STATES PATENT OFFICE.

FRED A. STIEF, OF EAST ST. LOUIS, ILLINOIS.

## REFINING LEAD ALLOYS AND ALLOYS CONTAINING LEAD, TIN, COPPER, OR ANTIMONY.

1,283,427.

Specification of Letters Patent. Patented Oct. 29, 1918.

Application filed May 6, 1915. Serial No. 26,207.

*To all whom it may concern:*

Be it known that I, FRED A. STIEF, a citizen of the United States, and a resident of the city of East St. Louis, county of St. Clair, 5 and State of Illinois, have invented a new and useful Improvement in Refining Lead Alloys and Alloys Containing Lead, Tin, Copper, or Antimony, of which the following is a specification.

10 This invention relates particularly to processes for removing arsenic from mixtures containing tin, antimony, lead and arsenic. No claim is made herein for the apparatus. The invention consists in exposing the molten mixture of metals to the action of iron, limestone or lime in a furnace, and separating the arsenic from the mixture in the form of speiss, which is composed largely of arsenic and iron or calcium in the form of 15 an arsenid or an arsenate. The operation is performed in a furnace of special design, wherein the metal is exposed to the action of the heat but protected from the action of the furnace gases, and which furnace may be equipped with a separator for 20 separating the speiss from the fluid metal.

Further details of the invention appear hereinafter, reference being had to the details of construction and operation of the 25 furnace shown in the accompanying drawings for purpose of illustration. What is claimed as the invention is defined in the appended claims. In the drawings, in which the same reference characters refer to like parts in the several views,

Figure 1 is a horizontal section through the furnace on the line 1—1 in Fig. 2, showing the hearth in plan;

Fig. 2 is a vertical longitudinal section 40 of the furnace on the line 2—2 in Fig. 1; and

Figs. 3 and 4 are vertical transverse sections of the furnace on the lines 3—3 and 4—4 in Fig. 2, respectively.

The furnace shown in the drawings comprises vertical side walls 10 inclosing a rectangular hearth 11 which is divided into three long narrow sections by means of longitudinal partition walls 12. The fire box 13 is at one end of the hearth and the chimney 14 is at the other end. The hearth and fire box are covered by tiles 15 which are supported on the side walls 10, partition walls 12 and front wall 16 of the furnace. The tiles are fitted with rings or loops 17 in their tops, by means of which they can be readily removed to give access to

the hearth. At each end of the hearth is a low cross wall 18 which retains the fluid metal on the hearth. The hot gases of the furnace pass over the cross walls 18 and above the hearth between the longitudinal walls 12, and a large part of the heat of the furnace gases is absorbed by these walls and by the roof tiles.

At one end of the hearth is an inlet or 65 charging duct 19 which leads through the side wall of the furnace from the hopper or trough 20 on the outside of the furnace. Molten metal may be run through this charging duct on to the hearth. The partition walls 12 are each provided at one end only with an opening 21. These openings connect the sections of the hearth between the partition walls. The opening 21 in one of the partition walls is at the opposite end 70 of the hearth from the opening 21 in the other partition wall, so that the fluid metal is obliged to travel the full length of the hearth between the partition walls in order to pass from one longitudinal division of 75 the hearth to the next.

At the opposite corner of the hearth from the inlet or charging duct is an outlet duct 22 which is provided with a spout 23 at the level of the hearth. In the bottom of the 85 hearth near the outlet end is an orifice 24 beneath which is arranged an iron receptacle or well 25. This well 25 constitutes a settling chamber for separating the fluid metal and the speiss, and it may be surrounded by a water jacket 26 through which 90 cooling water is caused to circulate by means of the pipes 27. At the bottom of the settling chamber 25 is a discharge duct 28 and tap hole 29.

Preferably the hearth is sloped from the charging duct slightly downward toward the outlet duct so that there will be a uniform fall for the molten metal throughout its course. This fall should not be too steep 100 as it is desirable that the metal should take one-half hour or more to flow from the inlet to the outlet duct in a wide thin stream of one-half inch or so in depth.

The process may be operated with any 105 suitable flux for removing the arsenic but a mixture of about one-half scrap iron and one-half charcoal or coke is preferable. The scrap iron and carbon are charged on to the hearth from above and are spread uniformly 110 along its entire length. The metal to be refined is charged on to the hearth in a molten

state, and as it flows slowly along the hearth it is filtered through the scrap iron and brought into intimate contact therewith. The charcoal or coke covers the molten metal and protects it from the furnace gases. The iron combines with the arsenic in the molten metal and forms "speiss," which is a fluid of lighter specific gravity than the molten metal. The speiss floats along with the metal to the outlet duct. The metal and speiss together float into the settling chamber, where the metal sinks to the bottom. When the settling chamber is full the speiss will flow out of the furnace through the outlet duct 22. The metal can be tapped off either continuously or at intervals from the bottom of the settling chamber through the discharge duct 28 and tap hole 29. The carbon and iron can be renewed from time to time as is required. The temperature of the furnace should be such as to maintain the metal and speiss at a red heat. The metal in the bottom of the separation chamber should be cooled to a temperature at which any speiss commingled therewith would solidify and float to the top.

In case a flux containing limestone or lime is used the arsenic and the calcium combine to form an arsenate which is not a fluid and which must be raked out of the furnace at intervals. This may be readily done by removing the tiles from over the hearth without interfering with the continuity of operation of the process. When lime or limestone is used in the flux either alone or in combination with other substances a sufficient amount of calcium-carbonate and calcium-arsenate may be left in the furnace as a cover for protecting the metal from the furnace gases.

Among the advantages of this process and apparatus are the following: The length of the path which the metal is caused to travel in its course over the hearth causes it to be thoroughly commingled with the flux which it passes, and the thinness of the layer treated insures that all parts of the metal are subjected to the same treatment. The partitions absorb a large part of the furnace heat and conduct it to the metal, and they also retain the flux on the hearth and keep it spread out uniformly. The process may be worked continuously and the flux may be renewed as required without requiring the furnace to be cooled off or cleaned out, the metal may be charged in continuously, and the metal and speiss may be tapped off continuously or intermittently as desired. The hearth is comparatively short and compact, the partitions support the roof and enable loose tiles to be used in place of a solid arch, and the loose tiles afford easy access to the hearth.

The settling chamber may be dispensed

with and instead the mixture of metal and speiss tapped off and cast in pigs, which are later remelted at a low heat to separate the metal from the speiss which has a higher melting point than the metal.

The invention is not restricted to the use of the ingredients and proportions above described.

I claim the following as my invention:

1. A process for refining alloys of lead, tin, copper, or antimony, containing arsenic which comprises treating the metal in a thin layer at a red heat in the presence of iron and separating out the speiss from the molten metal.

2. A process for refining alloys of lead, tin, copper, or antimony, containing arsenic which comprises treating the metal in a thin layer at a red heat in the presence of iron and calcium compound and separating out the speiss from the molten metal.

3. A process for refining alloys of lead, tin, copper, or antimony, containing arsenic which comprises treating the metal in a thin layer at a red heat in the presence of iron and separating out the speiss from the molten metal by cooling the mixture in a settling chamber.

4. A process for refining alloys of lead, tin, copper, or antimony, containing arsenic which comprises treating the metal in a thin layer at a red heat in the presence of iron and separating out the speiss from the molten metal by cooling the mixture in a settling chamber and removing the speiss from the top.

5. A process for refining alloys of lead, tin, copper, or antimony, containing arsenic which comprises treating the metal in a thin layer at a red heat in the presence of iron and separating out the speiss from the molten metal by freezing the speiss.

6. A process for refining alloys of lead, tin, copper, or antimony, containing arsenic which comprises treating the metal in a thin layer at a red heat in the presence of iron and carbon and separating out the speiss from the molten metal.

7. A process for refining alloys of lead, tin, copper, or antimony, containing arsenic which comprises treating the metal in a thin layer at a red heat in the presence of iron, calcium compound and carbon and separating out the speiss from the molten metal.

8. A process for continuously refining alloys of lead, tin, copper, or antimony, containing arsenic which comprises treating the metal in a thin layer at a red heat in the presence of iron and calcium compound in a furnace, renewing the iron from time to time and separating out the speiss containing iron from the molten metal while permitting the cinder containing calcium to remain in the furnace.

9. A process for continuously refining

- alloys of lead, tin, copper, or antimony, containing arsenic which comprises treating the metal in a thin layer at a red heat in the presence of iron and carbon in a furnace, renewing the iron and carbon from time to time and separating out the speiss from the molten metal by gravity.
10. The improvement in the process of refining alloys of lead, tin, copper, or antimony containing arsenic which comprises heating the metal in a thin layer in the presence of iron while maintaining a suitable material on top of the metal to prevent volatilization.
15. 11. A process for refining alloys of lead,
- tin, copper, or antimony containing arsenic which comprises heating the metal in a thin moving stream in the presence of iron while maintaining a sufficient amount of calcium compound to form a flux on top of the metal 20 to prevent volatilization.
12. A process for refining alloys of lead, tin, copper, or antimony containing arsenic which comprises heating the metal in the presence of iron in a thin moving stream 25 while maintaining a flux on top of the metal to prevent volatilization.

Signed at St. Louis, Missouri, this 3rd day of May, 1915.

FRED A. STIEF.